

## UNITED STATES PATENT OFFICE

2,147,125

## PRODUCTION OF LOW ARSENIC LIME

Henry V. Moss, St. Louis, Mo., assignor to Monsanto Chemical Company, a corporation of Delaware

No Drawing. Application August 14, 1937,  
Serial No. 159,098

4 Claims. (Cl. 23—186)

This invention relates to the production of a pure form of quick lime, and particularly to a form of quick lime having a low arsenic content.

I have found that in the ordinary method of burning lime in vertical kilns where coal is used as a fuel an appreciable amount of the arsenic present in the fuel becomes associated with the lime. I have also found that the arsenic thus associated with the lime remains in the surface layers of the lime lumps and that it may be substantially removed by partially hydrating and swelling the surface layers as by the addition of water or steam. Such treatment of lump lime results in the disintegration of the surface layer enabling said contaminated layer to be removed and separated from the core of the lime without effecting a substantial hydration of the latter.

As an example of the extent of arsenic contamination caused by a coal fuel, I have found that a typical hard burned lime will show an arsenic content upon the surface thereof at 4½ P. P. M. as  $As_2O_3$  whereas the layer of lime  $\frac{1}{2}$  inch in from the outside surface has an arsenic content of 1½ P. P. M. which is typical of the rest of the lime in the core. I have found that lime peeled off of the surface of lumps will in some cases run as high as 25 P. P. M.  $As_2O_3$ .

In the practise of my process I have found that the removal of the contaminated surface layers may be effected by abrasion as by tumbling the hard burned lumps of lime in a ball mill and removing the disintegrated powder which will contain a large proportion of the arsenic present in the lime. As a preferred method, however, I may treat the hard burned lump lime with such a proportion of water that a hydration of the surface layers of lime is effected. Such hydration results in a swelling and a formation of fairly uniform scales of hydrated lime which scales readily fall off of the lumps of lime leaving behind a uniform hard burned core having a relatively low ignition loss.

As an example of one method of practising my invention, I give the following description:

15 Limestone is charged to a vertical kiln and burned with an arsenic containing fuel such as coal until a hard-burned product is obtained. The lumps of limestone are so chosen as to be of maximum size, consistent with the production of a hard-burned product in the kiln employed and in any event should result in pieces of burned lime which are considerably larger than 1 inch mesh. I prefer to obtain lime averaging in the neighborhood of 4"-6" diameter pieces.

55 Upon discharging the burned product and cool-

ing in the usual way I pass the lump lime over say a 1 inch mesh shaking screen and spray the lime with a fine mist of water for say 1 minute. I may interrupt the spray for one minute to permit reaction of the water to take place. I repeat 5 the spraying with water at intervals say a total of say five times and then permit the lumps to stand for an additional period of 20 minutes. At the end of this time the screen is shaken to remove the loosely held partially hydrated outer 10 surface which has scaled off and which passes through the perforations in the screen. The centers of the lumps on the screen are essentially free of arsenic. In a typical experiment of this kind I have obtained the following arsenic values: 15

Arsenic in original quick lime, 1.4 P. P. M. bone dry basis.

Arsenic in outer surface lime, 3.0 P. P. M. bone dry basis.

Arsenic in centers held on screen, 0.6 P. P. M. 20 bone dry basis.

In this experiment, the outer surface which was removed represents 27% of the original quick lime, thus leaving 73% of the lime essentially arsenic free. The outer surface is partially hydrated by the water to a lime having an ignition 25 loss of 9½% while the inner cores show an ignition loss of only 4.8%.

The high arsenic partially hydrated portion 30 may be disposed of thru any suitable means where arsenic contamination or the need of moisture-free quick lime is not a factor, as for instance in the building industry or as agricultural lime.

The low arsenic lime obtained by my process 35 may be used in the manufacture of lime containing food products and wherever a low arsenic content is necessary.

The amount of lime removed from the outer 40 surface of the burned lumps will depend somewhat upon the size of the lumps and upon the arsenic content thereof. It is therefore subject to some variation dependent upon these factors.

Having described my invention, what I claim 45 is:

1. The process of decreasing the arsenic content of lump lime which has been burned with arsenic containing fuels comprising disintegrating the outer surface of said lumps and separating the disintegration product from the remaining lumps.

2. The process of decreasing the arsenic content of lump lime which has been burned with arsenic containing fuels comprising disintegrating the outer surface of said lumps by the appli- 55

cation of water thereto and separating the disintegration products from the remaining lumps.

3. The process of producing substantially arsenic-free lime comprising hard-burning limestone lumps with arsenic containing fuels, cooling the hard burned lumps of lime and then disintegrating and removing the outer surface thereof.

4. The process of producing substantially arsenic-free lime comprising hard burning limestone lumps with a coal fuel and obtaining thereby hard-burned lime lumps having an outer shell of high arsenic lime and then removing said outer shell by disintegration. 5

HENRY V. MOSS.